

# United States Patent

Tabor et al.

[15] 3,658,575

[45] Apr. 25, 1972

[54] **METHOD AND COMPOSITIONS FOR TREATING FLEXIBLE SUBSTRATES**

[72] Inventors: **Theodore E. Tabor; Hugh A. Farber; Thomas A. Vivian, all of Midland, Mich.**

[73] Assignee: **The Dow Chemical Company, Midland, Mich.**

[22] Filed: **Sept. 29, 1969**

[21] Appl. No.: **862,031**

[52] **U.S. Cl. .... 117/102 R, 117/135.5, 117/136, 117/139.4, 117/139.5**

[51] **Int. Cl. .... B05c 11/10, B05c 3/18**

[58] **Field of Search .... 117/102 R, 63, 139.4, 135.5, 117/139.5 R, 119.8, 102 A, 121, 66, 136; 260/29.4 R, 33.8 R**

[56] **References Cited**

UNITED STATES PATENTS

|           |        |                      |             |
|-----------|--------|----------------------|-------------|
| 2,373,135 | 4/1945 | Maxwell.....         | 117/139.4 X |
| 2,731,364 | 1/1956 | Reibnitz et al. .... | 117/161 X   |
| 3,023,129 | 2/1962 | Hersh et al. ....    | 117/139.4   |

*Primary Examiner—Murray Katz  
Assistant Examiner—Theodore G. Davis  
Attorney—Griswold & Burdick, Giwynn R. Baker and C. E. Rehberg*

[57] **ABSTRACT**

A process for applying water-soluble chemicals to flexible substrates, e.g., textile fibers, yarns, non-woven, loomed, tufted woven and knit materials, paper and the like, which employs a readily removable carrier formulation at lower temperatures under ambient pressures consisting of preparing an aqueous-oil emulsion of the chemical and its attendant assistants, catalysts or reactive or non-reactive co-chemicals, surface active agent(s) in 1 to 35 percent by weight water and 98 to 40 percent by weight of a halogenated hydrocarbon solvent boiling between about 40° to about 165° C., applying the emulsion to a flexible substrate by dipping, immersing, flooding, doctoring, spraying or the like, introducing the so-wetted substrate into a zone filled with the vapors of the halogenated solvent which is at a temperature at or above the boiling point of the solvent of the emulsion, maintaining the substrate in said vapors for a time sufficient to remove the water and solvent from the substrate, and removing the substrate from said zone in a dry condition retaining the chemical(s) thereon or in.

5 Claims, No Drawings

## METHOD AND COMPOSITIONS FOR TREATING FLEXIBLE SUBSTRATES

### BRIEF DESCRIPTION OF INVENTION

In accordance with the present invention, a flexible substrate such as, for example, a textile fiber, yarn, knit, loomed or woven fabric or cellulose fiber, paper, etc., is treated with a water-in-oil emulsion of a treating agent or mixture of treating agents from a 1 to 30 percent by weight water and 99 to 40 percent by weight halogenated emulsified carrier by applying the emulsion to the flexible substrate by dipping, spreading, immersing, flooding, spraying or the like; introducing the wetted substrate into a zone filled with the vapors of a halogenated solvent boiling between about 40° and about 165° C. which zone is maintained at or above the boiling point of the solvent employed in the emulsion; maintaining the substrate in said zone until the solvent has been removed; and finally withdrawing the substrate from the zone in a dry condition retaining the treating chemical.

The nature of the substrate is not critical and may be derived from natural or synthetic fibers and may be in the form of yarns, threads, films, sheets, woven, unwoven, loomed, or the like. The commonly employed fibers are or derived from flax, cotton, wood, jute, polyamide, polyester, polyacrylate and polyarylonitrile and mixtures thereof. These fibers may be chemically treated as in the case of cellulose to enable their reforming as fibers, strands, threads or films. Mixtures of two or more fibers from each class may be combined.

The halogenated hydrocarbon solvents useful in accordance with the present invention are those having a boiling point

and resins, fire retardants and the like. Representative of such chemicals are the methylol or alkyl ethers of methylol compounds (dimethylol dihydroxyethylene ureas), the silicones, the fluorocarbon stain and water repellents, fluorocarbon stabilization and wrinkle resistant resins, polyethylenes, polyglycols and the inorganic salts used for fire retardance.

### DETAILED DESCRIPTION OF INVENTION

#### EXAMPLE 1

A 100 percent cotton 80 × 80 print cloth was treated by spraying one of the compositions as set forth in the following tables, the solvent and water removed by passing the wetted fabric through a zone of vapors of stabilized 1,1,1-trichloroethane while simultaneously passing the fabric over two heated cans (internal steam pressure ca 60 psi). The fabric was passed through the vapor zone at ca 10 yards per minute, residence time about 12 seconds. The fabric was dry, neither wet with moisture of solvent upon being withdrawn from the vapor zone.

The fabric was after-cured for 5 minutes at 150° C. and the wrinkle recovery angle measured according to AATCC 66-1968 Monsanto Wrinkle Recovery Test. Durable press was measured by AATCC 124-1967. Tensile change and elongation change were both measured on an Instron Tensile Instrument, five samples run each direction and averaged. AATCC 30 88C1964 was employed to obtain crease retention values.

The control runs using only water as the formulation carrier were made in the same equipment but without the vapor zone.

TABLE I

| Formulation percent by weight based on total weight of formulation |       |                                            |                                  |             |         |                                                                   | Wrinkle recovery angle, degrees | Durable press |
|--------------------------------------------------------------------|-------|--------------------------------------------|----------------------------------|-------------|---------|-------------------------------------------------------------------|---------------------------------|---------------|
| Dimethylol dihydroxy-ethylene urea                                 | Water | Zn(NO <sub>3</sub> ) <sub>2</sub> catalyst | Commercial polyethylene softener | Surfactant* | Solvent | Percent resin solids added on after drying solids wt./fabric wt.) |                                 |               |
| 4-----                                                             | 12    | 0.6                                        | 1.0                              | 1.0         | 81.4    | 6.1                                                               | 279                             | 3.3           |
| 4-----                                                             | 8     | 0.6                                        | 1.0                              | 1.0         | 85.4    | 6.4                                                               | 280                             | 3.0           |
| 3-----                                                             | 6.7   | 0.45                                       | 1.0                              | 1.0         | 87.8    | 5.5                                                               | 265                             | 3.2           |
| 5-----                                                             | 91.8  | 0.75                                       | 1.25                             | 1.25        | 0       | 4.6                                                               | 262                             | 3.3           |
| Untreated control                                                  |       |                                            |                                  |             |         |                                                                   | 169                             | 1.0           |

\*Dioctyl sodium sulfo succinate.

The tensile change in percent and elongation change in percent are set forth in the following table.

between about 40° and 165° C., single species of halogen or mixtures of halogen, saturated or ethylenically unsaturated. Thus, the chlorinated methanes, chlorinated ethanes, the 50 fluorinated ethanes, the mixed fluorochloro and fluorobromo ethanes and the like. Representative of the preferred classes of halogenated hydrocarbons falling within these classes are methylene chloride, chloroform, carbon tetrachloride, 1,1,1-trichloroethane, trichloroethylene, perchloroethylene; dichromotetrachloroethane, tetrachlorodifluoroethane, dichlorotetrafluoroethane, trichlorotrifluoroethane and the like.

The classes of treating agents which can be applied by the 60 method of the present invention is very broad. For example, durable press resins, water repellent resins and chemicals, stain repellent chemicals, fiber stabilization resins, dyes, softeners, lubricants, soil release chemicals, finishing chemicals

In another series of experiments, a 65/35 polyester cotton broadcloth shirting fabric was treated in the same manner as set forth in Example 1 using the formulations set forth in Table II. The durable press rating and crease resistance were measured and are set forth in the Table.

TABLE I(a)

| Warp     | Fill | Elongation change, percent |      |
|----------|------|----------------------------|------|
|          |      | Warp                       | Fill |
| -47----- | -50  | -49                        | -26  |
| -40----- | -46  | -39                        | -29  |
| -41----- | -48  | -34                        | -38  |
| -53----- | -53  | -48                        | -26  |

#### EXAMPLE 2

TABLE II

| D.P. resin         | Water | Percent by weight                    |          |            |            | Percent added on | Durable press rating | Crease resistance | Sum DP+CR |
|--------------------|-------|--------------------------------------|----------|------------|------------|------------------|----------------------|-------------------|-----------|
|                    |       | Catalyst (15% based on resin solids) | Softener | Surfactant | Solvent    |                  |                      |                   |           |
| 6-----             | 11    | 0.9                                  | 1.0      | 1.0        | Balance .. | 5.0              | 3.5                  | 4.2               | 7.7       |
| 8-----             | 14    | 1.2                                  | 1.0      | 1.0        | Balance .. | 8.2              | 3.3                  | 3.8               | 7.1       |
| 10-----            | 16    | 1.5                                  | 1.0      | 1.0        | Balance .. | 10.3             | 3.5                  | 4.4               | 7.9       |
| 7.5-----           | Bal.  | 1.125                                | 1.0      | -----      | -----      | 4.9              | 3.4                  | 4.1               | 7.5       |
| 9.8-----           | Bal.  | 1.47                                 | 1.0      | -----      | -----      | 6.0              | 3.6                  | 4.4               | 7.4       |
| 12-----            | Bal.  | 1.8                                  | 1.0      | -----      | -----      | 7.6              | 3.6                  | 3.8               | 7.4       |
| Control, untreated |       |                                      |          | -----      | -----      | -----            | 2.5                  | 2.6               | 5.1       |

## EXAMPLE 3

A durable press resin (dimethylol dihydroxyethylene urea) and either a silicone water repellent resin or a fluorocarbon water and stain repellent resin were applied from a formulation within the teaching of the present invention to a 50/50 polyester-cotton poplin fabric. The fabric was wetted with formulation to about 50% wet pick-up in a Butterworth 15 inch Laboratory Padder, 1 dip 1 nip. The results of these operations are set forth below.

The formulations employed were:

A. 10% by weight dimethylol dihydroxyethylene urea (DMDHEU), 1.5%  $Zn(NO_3)_2$ , 1% polyethylene, 2% DC 1109 silicone, 15.8% water and 69.7% 1,1,1-trichloroethane.

B. 10% (DMDHEU)

1.5%  $Zn(NO_3)_2$

1% Polyethylene

2% DC 1172 silicone

0.1% DC catalyst XY-168

15.1%  $H_2O$

70.3% 1,1,1-Trichloroethane

C. 10% DMDHEU

1.5%  $Zn(NO_3)_2$

1% Polyethylene

0.63% Fluorocarbon FC 208

15.8% Water

71.1% 1,1,1-Trichloroethane

5

Cotton  
Polyester  
Polyester-Cotton

10

4  
TABLE V

| Resin Application | % Removed by Solvent Wash |
|-------------------|---------------------------|
| Aqueous           | 0                         |
| Emulsion          | 3                         |
| Aqueous           | 68                        |
| Emulsion          | 61                        |
| Aqueous           | 16                        |
| Emulsion          | 25                        |

Hand of the washed fabric was softer than non-solvent washed controls.

15

## EXAMPLE 6

A paste was made by mechanically mixing 25 percent of a commercial carpet backsizing compound and 75 percent 1,1,1-trichloroethane. The carpet backsizing compound used was 65 percent solids in water. The solids portion consists of 100 parts styrene-butadiene latex and 350 parts calcium carbonate. An even coat of the above paste was applied to a piece of carpeting 4 inches by 3 inches using a brush. In commercial applications, such materials are generally applied by roll coat followed by a doctor blade. The initial weight increase on the carpet sample was approximately 140 percent. The treated carpet sample was then dried by laying it on a hot metal surface at 250°F. with the pile side contacting the metal surface. The sample dried quite rapidly and was weighed periodically

TABLE III

| Formulation    | Percent add-on resin wt./ fabric wt. | WRA° | Spray rating |        |          | Oil rating |        |
|----------------|--------------------------------------|------|--------------|--------|----------|------------|--------|
|                |                                      |      | Initial      | 1 Wash | 5 Washes | Initial    | 1 Wash |
| A-----         | 7.9                                  | 298  | 100          | 90     | -----    | 1          | 1      |
| B-----         | 7.1                                  | 311  | 100          | 100    | 80       | -----      | -----  |
| C-----         | 7.7                                  | 309  | 100          | 80     | -----    | 5          | 4      |
| Untreated----- | -----                                | 217  | 0            | 0      | -----    | 1          | 1      |

## EXAMPLE 4

In another series of experiments, the effect of conditioning of the fabric with steam after curing was determined.

100 percent 80 x 80 cotton print cloth was sprayed with a formulation consisting of:

8% N,N'-bis(methoxymethyluron)  
1.2%  $ZnCl_2$   
3.6% Ethanol  
87.2% 1,1,1-Trichloroethane.

The wetted fabric was air dried. The fabric, found to have about a 7.6 percent add-on of resin, was steamed at atmospheric pressure, then cured at 160°C. for 5 minutes. The results of the runs are set forth below:

TABLE IV

| Steaming Time (Min.) | WRA° |
|----------------------|------|
| 0.5                  | 261  |
| 1.0                  | 263  |
| 2.0                  | 263  |
| 3.0                  | 260  |
| 4.0                  | 257  |
| Untreated 4.0        | 157  |

## EXAMPLE 5

In another series of experiments, the effect of solvent washing prior to cure was determined. The nature of the treating formulation and treatment technique was as set forth in Example 1 using cotton print cloth, polyester plain weave and polyester-cotton batiste. The washing was conducted for 20 minutes in 1,1,1-trichloroethane containing 0.0045 percent by weight diethylsodiumsulfosuccinate, rinsed twice for 10 minutes in 1,1,1-trichloroethane and air dried. The amount of resin lost is recorded below:

40 during the drying process. The sample was dry after approximately 25 minutes as there was little additional weight loss after this period. The sample weight at this point indicated a backsizing add-on of approximately 25 percent on the initial weight of the sample. This technique gave a good uniform coating on the carpet sample.

We claim:

1. A process for the application of water-soluble durable press resins, water repellent resins and chemicals, stain repellent chemicals, fiber stabilization chemicals, dyes, softeners, lubricants, soil release chemicals, finishing chemicals and resins on fire retardant, or mixtures thereof to a flexible substrate of natural and synthetic fibers and yarns, threads, films sheets thereof woven, unwoven or loomed which comprises: applying the chemicals to the flexible substrate from an aqueous emulsion carrier which contains 1 to 35 percent by weight water based on the total weight of the emulsion, 98 to 40 percent by weight of a halogenated hydrocarbon solvent having a boiling point between about 40° and 165°C., the treating chemicals being present in from 0.2 to 15 percent by weight; introducing the wetted substrate into a zone filled with vapors of a halogenated solvent having a boiling point between about 40° and 165°C. which is at or above the boiling point of the halogenated hydrocarbon solvent employed in the emulsion; maintaining the substrate in said zone until the halogenated hydrocarbon solvent and water are removed from the substrate; and, withdrawing the substrate from the zone free of water and halogenated hydrocarbon solvent.

2. The process of claim 1 wherein said flexible substrate is a textile fabric, said chemicals are a durable press resin of the class methylol and alkyl ethers of methylol compounds, a catalyst for said resin and said halogenated hydrocarbon is the same solvent as that employed to fill the vapor zone.

3. The method of claim 2 wherein the substrate is steamed

at atmospheric pressure for from 0.5 to 4 minutes, then heated at from 150° - 160° C. to cure the resin.

4. The process of claim 2 wherein said resin is dimethylol

dihydroxyethylene urea and the catalyst is  $Zn(NO_3)_2$ .

5. The process of claim 2 wherein said resin is N,N'-bis(methoxymethyl)uron and the catalyst is zinc chloride.

\* \* \* \* \*